

Dec. 6, 1932.

R. S. DEAN

1,890,013

LEAD ALLOY

Filed June 29, 1928



Inventor  
Reginald S. Dean  
by A. A. Johnson Att'y.

## UNITED STATES PATENT OFFICE

REGINALD SCOTT DEAN, OF RIVERSIDE, ILLINOIS, ASSIGNOR TO WESTERN ELECTRIC COMPANY, INCORPORATED, OF NEW YORK, N. Y., A CORPORATION OF NEW YORK

## LEAD ALLOY

Application filed June 29, 1928. Serial No. 289,145.

This invention relates to lead alloys, articles made therefrom, and methods of producing and/or treating such alloys and articles, and more particularly to alloys of lead and calcium, extruded articles made therefrom, and methods of producing and/or treating such alloys and articles.

An object of the invention is to provide alloys of lead and calcium having some or all of the properties of extreme hardness, high tensile strength, great resistance to failure from fatigue, large percentage elongation, excellent resistance to corrosion, and great stability at atmospheric temperatures.

Another object of the invention is to provide articles made of alloys of lead and calcium, particularly electrical cable sheaths made of such alloys.

Additional objects of the invention are to provide simple, effective, and expeditious methods of producing and/or treating alloys of lead and calcium and articles made from such alloys resulting in and having desired physical and mechanical properties.

In accordance with the general features of the invention as embodied in one specific form thereof, a quantity of calcium is alloyed with a sufficient quantity of lead to produce an alloy containing less than 1% calcium and the alloy caused to solidify. The solidified alloy is heated at a temperature sufficiently high and for a sufficiently long period of time to cause substantially all of the resulting solute constituent to enter solid solution in the lead, and the alloy is then cooled from an elevated temperature at a sufficiently rapid rate to cause some of the solute constituent to remain in the lead in the form of a supersaturated solid solution, after which the alloy is caused to assume a more stable state by aging. In the manufacture of articles, such as cable sheaths, from an alloy of the type just described, an article may be formed therefrom and then the formed article subjected to the above outlined heating, cooling and aging operations, or else the alloy may be first reduced to the form of a solid solution and an article produced therefrom while

the alloy is hot, after which the hot article

is cooled and aged in the manner described above.

The above described and other objects and features of the invention will be apparent from the following detailed description of one embodiment of the invention, taken in connection with the accompanying drawing, in which

Fig. 1 is an equilibrium diagram of the lead-rich end of the lead-calcium system;

Fig. 2 is a diagram showing the comparative tensile strengths of alloys treated in accordance with this invention and alloys not so treated, and

Fig. 3 is a diagram similar to that shown in Fig. 2 showing the comparative percentage elongations of treated and untreated alloys.

Referring now to Fig. 1 of the drawing, the curves shown therein represent the loci of the points at which transformations in the physical conditions of lead-rich alloys of lead and calcium occur. In the diagram shown in Fig. 1, the temperatures at which the transformations occur are plotted as ordinates and the percentage compositions of the alloys in which the transformations occur are plotted as abscissæ. The curve ABC in the diagram is a liquidus curve from which the melting points of the various lead-calcium alloys may be obtained, while the curve DE represents the solubility in lead of the solid solute constituent separating out with the lead when the alloys solidify. From an examination of the diagram it will be seen that the solubility of the solid solute constituent in lead varies with the temperature, the solid lead dissolving about .1% of the calcium at 330° C. and less than .02% at room temperature or lower temperatures. In accordance with this invention, advantage is taken of the above described characteristics of lead-rich alloys of lead and calcium to produce alloys having enhanced properties and to produce articles, such as cable sheaths, from these alloys.

Although it is not known with certainty just what the solution of the lead and the solute constituent comprises, it is believed that the calcium combines chemically with a part of the lead to form a compound having

the formula  $Pb_8Ca$  which enters solid solution in the remainder of the lead and separates out as a distinct constituent under certain conditions. In any event, whether or not such a compound is found, the calcium, either combined or uncombined chemically with a part of the lead, enters into solid solution in the lead. The theory upon which the processes described below are based is the same regardless of whether the calcium is free or combined and it is to be understood, therefore, that in the following description and annexed claims when it is stated that the solute constituent or the calcium is caused to enter solid solution in the lead, these terms are intended to mean either combined or uncombined calcium as the case may actually be.

In practicing one method of producing alloys in accordance with the invention, a quantity of calcium falling within the range bounded by the maximum amount of calcium which will enter solid solution in lead at any temperature at which the resulting alloy is a solid and the amount of calcium which will be retained in solid solution in lead at room temperature (.02% to .1% calcium) is alloyed with lead and the resulting alloy caused to solidify. The solid alloy is then heated at a temperature sufficiently high to cause the calcium to enter solid solution in the lead, which temperature may be determined by referring to the diagram shown in Fig. 1 of the drawing, and the heating is continued until substantially all of the calcium has entered into a substantially homogeneous solid solution in the lead. The alloy is then cooled from an elevated temperature at a rate sufficiently rapid to insure the retention of some of the calcium in the lead in the form of a supersaturated solution, after which the alloy is caused to assume a more stable state by aging. The percentage of calcium employed and the temperatures at which the heating, cooling and aging steps are practiced depend upon the characteristics desired in the finished product and may be determined by reference to Figs. 2 and 3 of the drawing.

Referring now to Fig. 2 of the drawing, which illustrates the comparative tensile strengths of alloys treated in accordance with the invention and alloys not so treated, the curve F represents the tensile strength of the various alloys, whose compositions are indicated as abscissæ, which have been heated at a temperature of approximately  $320^{\circ} C.$  until a substantially homogeneous solid solution was produced and quenched from the temperature of  $310^{\circ} C.$  to room temperature and aged at room temperature, while the curve G illustrates the tensile strengths of corresponding alloys which have been slowly cooled from  $310^{\circ} C.$  to room temperature so that practically no supersatura-

tion of the solution of the solute constituent in the lead results. It will be seen by reference to Fig. 2 that the alloys treated in accordance with the invention possess considerably greater tensile strength than is possessed by the alloys not so treated, and also that the tensile strength of the treated alloys varies with the composition thereof, the tensile strength reaching a high value when an alloy containing about .1% calcium is employed. From this it will be evident that great tensile strength in the treated alloys results when the maximum amount of calcium which will enter solid solution in lead at any temperature at which the resulting alloy is a solid is employed.

Referring now to Fig. 3 of the drawing which illustrates the comparative percentage elongations of alloys treated in accordance with the invention and alloys not so treated, the curve H represents the percentage elongations in six inches of alloys which have been formed into a solid solution, reduced to a supersaturated solid solution and aged, while the curve I represents the percentage elongations of corresponding alloys which have been produced in such a manner that vary little, if any, supersaturation of the solid solution results. As a general rule, the percentage elongation of metals decreases rapidly with increased tensile strength and it might be expected that lead-calcium alloys of increased tensile strength would exhibit low percentage elongations. However, from an examination of these curves it will be apparent that the percentage elongations of the treated alloys, while less than those obtained in the untreated alloys, are not sufficiently less to materially decrease the usefulness of the treated alloys for the manufacture of articles, such as cable sheaths. As in the case of the tensile strength, a high percentage elongation results when the maximum amount of calcium is employed which will enter solid solution in lead at any temperature at which the resulting alloy is a solid, namely about .1% calcium.

If an alloy of a particular tensile strength and percentage elongation is desired, these characteristics may be obtained by employing an alloy having the composition corresponding to the particular characteristics desired. For instance, if it is desired to produce an alloy having a tensile strength of about 7000 pounds per square inch and a percentage elongation of about 40%, approximately .1% calcium is alloyed with lead and the resulting alloy is reduced to a solid state. The solid alloy is then heated at a temperature between  $310$  and  $325^{\circ} C.$ , which is the temperature necessary to cause this quantity of calcium to enter solid solution in lead, and the heating is continued until substantially all of the calcium has entered solid solution in the lead. If great tensile strength is de-

sired, the alloy is quenched from a temperature of about 310° C. to room temperature by immersing the alloy in water, and the alloy is caused to assume a more stable state by 5 aging the alloy at a temperature at which little agglomeration occurs, room temperature having proven to be a very satisfactory temperature at which to conduct the aging step. By the above described process an 10 alloy is produced consisting of a matrix of lead throughout which are substantially uniformly dispersed a large number of minute particles containing calcium and it is believed that the enhanced properties which 15 such alloys possess result from the wide dispersion of these particles and the extreme minuteness of the particles. It is important, therefore, that the aging step be carried on at a temperature sufficiently low so that little 20 agglomeration of the finely dispersed particles results, and it has been found that little agglomeration occurs when the alloy is aged at a temperature below 150° C.

By practicing the above outlined method, 25 alloys having very desirable properties may be produced. For instance, alloys having a tensile strength from 4000 to 7000 pounds per square inch, a percentage elongation of from 25 to 40% and a fatigue limit of from 800 to 30 1900 pounds per square inch, may be obtained by following the above outlined process. Other advantageous properties of such alloys are their resistance to chemical corrosion and their extreme stability of physical 35 properties at atmospheric temperatures.

The above enumerated properties of alloys produced in accordance with this invention are very desirable in extruded articles, particularly sheaths for electrical cables, and 40 the above described process provides an excellent means for producing such articles. For instance, in the manufacture of electrical cable sheaths, a lead-calcium alloy of the composition necessary to give the tensile 45 strength, percentage elongation, etc., desired in the finished sheath is produced, and the solid alloy then heated and extruded in the form of a sheath surrounding an electrical cable under such conditions that the alloy 50 making up the sheath as extruded will be in the form of a substantially homogeneous solid solution. The alloy is then cooled at a rate sufficiently rapid to insure the retention 55 of some of the solute constituent in a supersaturated solution in the lead and the sheath then aged to cause a dispersion of a solute constituent throughout the lead in the form of minute particles. Electrical cable sheaths 60 made in accordance with the invention have proven to have characteristics far superior to those made of other alloys commonly used in the manufacture of cable sheaths, and consequently sheaths made in accordance with 65 the invention will be much more effective

under service conditions than those heretofore known to the art.

It is, of course, to be understood that the methods outlined above and the articles and alloys produced by practicing these methods 70 are merely illustrations of useful embodiments of the invention and the invention is limited only by the scope of the annexed claims.

What is claimed is:

1. A method of producing improved alloys of lead, which consists in alloying calcium therewith, heating the alloy to form a solid solution, cooling the alloy to produce a supersaturated solid solution, and aging the alloy 80 to cause the dispersion of minute particles containing the calcium substantially uniformly throughout the lead.

2. A method of producing improved alloys of lead, which consists in alloying calcium 85 therewith, heating the alloy to form the same into a substantially homogeneous solid solution, cooling the alloy from an elevated temperature at a rate sufficiently rapid to insure the retention of calcium in the lead in the 90 form of a supersaturated solid solution, and aging the alloy to cause it to assume a more stable state.

3. A method of producing improved lead 95 alloys, which consists in alloying with lead a quantity of calcium falling within the range bounded by the maximum amount of calcium which will enter solid solutions in lead at any temperature at which the resulting alloy 100 is a solid and the amount of calcium which will remain in solid solution with lead at room temperature, forming the resulting alloy into a solid solution, reducing the alloy to a supersaturated solid solution, and aging the alloy to cause it to assume a more stable 105 state.

4. A method of producing improved alloys of lead, which consists in alloying from .02 to .1% calcium therewith, forming the alloy 110 into a supersaturated solid solution, and aging the resulting alloy to cause the dispersion of minute particles containing the calcium substantially uniformly throughout the lead.

5. A method of producing improved alloys of lead, which consists in alloying about .1% calcium therewith, forming the resulting alloy into a solid solution, reducing the alloy to a supersaturated solid solution, and aging the alloy to cause it to assume a more stable 115 state.

6. An alloy of lead and calcium, characterized by the presence of minute particles containing the calcium substantially uniformly dispersed through the lead, the metallurgical structure being formed by heating the alloy 120 to form it into a solid solution, reducing the alloy to a supersaturated solid solution, and aging the alloy.

7. An alloy of lead and calcium containing a quantity of calcium falling within the 125

range bounded by the maximum amount of calcium which will enter solid solution in lead at any temperature at which the resulting alloy is a solid and the amount of calcium which will be retained in solid solution in lead at room temperature, and characterized by the presence of minute particles containing the calcium substantially uniformly dispersed throughout the lead, the metallurgical structure being formed by heating the alloy to form it into a solid solution, reducing the alloy to a supersaturated solid solution, and aging the alloy.

8. An alloy of lead and calcium containing from .02 to .1% calcium, and characterized by the presence of minute particles containing the calcium substantially uniformly dispersed throughout the lead, the metallurgical structure being formed by heating the alloy to form it into a solid solution, reducing the alloy to a supersaturated solid solution, and aging the alloy.

9. An alloy of lead and calcium wherein the calcium is uniformly dispersed having a tensile strength of from 4000 to 7000 pounds per square inch, a percentage elongation greater than 30% in six inches, and a fatigue limit of from 800 to 1900 pounds per square inch, the metallurgical structure being formed by heating the alloy to form it into a solid solution, reducing the alloy to a supersaturated solid solution, and aging the alloy.

10. An age-hardened alloy of lead and calcium containing a quantity of calcium falling within the range bounded by the maximum amount of calcium which will enter solid solution in lead at any temperature at which the resulting alloy is a solid and the amount of calcium which will be retained in solid solution in lead at room temperature, the metallurgical structure being formed by heating the alloy to form it into a solid solution, reducing the alloy to a supersaturated solid solution, and aging the alloy.

11. An age-hardened alloy of lead and calcium containing from .02 to .1% calcium, the metallurgical structure being formed by heating the alloy to form it into a solid solution, reducing the alloy to a supersaturated solid solution, and aging the alloy.

12. An age-hardened alloy of calcium and lead containing substantially .1% calcium, the metallurgical structure being formed by heating the alloy to form it into a solid solution, reducing the alloy to a supersaturated solid solution, and aging the alloy.

13. A method of producing improved alloys of lead, which consists in alloying calcium therewith, heating the resulting alloy to form it into a solid solution, reducing the alloy to a supersaturated solid solution, and aging the alloy to cause it to assume a more stable state.

14. A method of producing improved alloys of lead, which consists in alloying cal-

cium therewith, heating the alloy to form the same into a substantially homogeneous solid solution, reducing the alloy to a supersaturated solid solution, and aging the alloy.

15. A method of producing improved alloys of lead, which consists in alloying calcium therewith, heating the alloy at a temperature slightly below the fusion temperature thereof until a substantially homogeneous solid solution is produced, reducing the alloy to a supersaturated solid solution, and aging the alloy.

16. A method of producing improved alloys of lead, which consists in alloying calcium therewith, heating the alloy at a temperature of 280° C. to 320° C. until a substantially homogeneous solid solution is formed, cooling the alloy at a rate sufficiently rapid to insure the retention of calcium in the lead in the form of a supersaturated solid solution, and aging the alloy to cause it to assume a more stable state.

17. A method of producing improved lead alloys, which consists in alloying with lead a quantity of calcium falling within the range bounded by the maximum amount of calcium which will enter solid solution in lead at any temperature at which the resulting alloy is a solid and the amount of calcium which will remain in solid solution in lead at room temperature, heating the alloy to form a solid solution, cooling the alloy to produce a supersaturated solid solution, and aging the alloy to cause the dispersion of minute particles containing the calcium substantially uniformly throughout the lead.

18. A method of producing improved alloys of lead, which consists in alloying from .02% to .1% calcium therewith, heating the resulting alloy to form it into a solid solution, reducing the alloy to a supersaturated solid solution, and aging the alloy to cause it to assume a more stable state.

19. A method of producing improved alloys of lead, which consists in alloying therewith substantially the maximum amount of calcium which will enter solid solution in lead at any temperature at which the resulting alloy is a solid, heating the alloy to form a solid solution, cooling the alloy to form a supersaturated solid solution, and aging the alloy to cause the dispersion of minute particles containing the calcium substantially uniformly throughout the lead.

20. A method of producing improved alloys of lead, which consists in alloying therewith substantially the maximum amount of calcium which will enter solid solution in lead at any temperature at which the resulting alloy is a solid, heating the resulting alloy to form into a solid solution, reducing the alloy to a supersaturated solid solution, and aging the alloy to cause it to assume a more stable state.

21. A method of producing improved al-

loys of lead, which consists in alloying about .1% calcium therewith, heating the alloy to form a solid solution, cooling the alloy to form a supersaturated solid solution, and 5 aging the alloy to cause the dispersion of minute particles containing the calcium substantially uniformly throughout the lead.

22. An alloy of lead and calcium containing substantially .1% calcium, and characterized by the presence of minute particles containing the calcium substantially uniformly dispersed throughout the lead, the metallurgical structure being formed by bringing the alloy into solid solution, reducing the 10 alloy to a supersaturated solution, and aging the alloy.

23. The method of producing a lead alloy, which comprises alloying with a quantity of lead a quantity of calcium greater than is 20 soluble therein at room temperature, maintaining the alloy at an elevated temperature below its melting point to cause the calcium to enter solid solution in the lead, quickly reducing the temperature of the alloy to form 25 a supersaturated solid solution, and aging the alloy to cause dispersion of minute particles containing calcium substantially uniformly throughout the lead.

In witness whereof, I hereunto subscribe  
80 my name this 7th day of June, A. D. 1928.  
REGINALD SCOTT DEAN.

35

40

45

50

55

60

65